

## UNITED STATES PATENT OFFICE

CHAD H. HUMPHRIES, OF INDIANAPOLIS, INDIANA, ASSIGNOR TO JAMES C. PATTEN, OF INDIANAPOLIS, INDIANA; E. KIRK MCKINNEY SPECIAL ADMINISTRATOR OF SAID JAMES C. PATTEN, DECEASED

## CADMIUM PLATING BATH

No Drawing.

Application filed April 4, 1928. Serial No. 267,273.

The object of my invention is to secure a bright homogeneous and coherent electrolytic plating of cadmium upon another metal.

I have discovered that the desired result 5 may be accomplished by adding to an acid cadmium plating bath commercial barley sugar, cane sugar caramel or malt sugar or malt syrup.

For instance in an acid plating bath having 10 two and one-half ounces of cadmium oxide and six ounces of sulphuric acid per gallon of water one to ten grams of one of the sugars mentioned above will insure a fine lustrous, dense, homogeneous deposit of cadmium.

The same is true in an acid bath containing 15 two and one-half ounces of cadmium oxide, six ounces of sulphuric acid and four ounces of ammonium sulphate per gallon of water.

Similar baths can be produced by dissolving 20 in water a dry mixture composed of two and one-half to three ounces of cadmium oxide, six ounces of acid sodium sulphate and four ounces of ammonium sulphate, or a mixture 25 of four ounces of cadmium sulphate and six ounces of ammonium sulphate, per gallon of water.

Where the dry mixtures mentioned above 30 are used in producing the bath, the desired quantity, one to ten grams, of the glucoside brightener may be preliminarily associated with the dry ingredients if desired.

I claim as my invention:

1. That improvement in the art of cadmium plating which involves the inclusion, 35 in an appropriate bath containing cadmium oxide and sulphuric acid, in the approximate proportions of 2½ ounces of cadmium oxide and 6 ounces of sulphuric acid per gallon of water, of 1 to 10 grams of commercial cane sugar caramel.

2. That improvement defined in claim 1 40 wherein the bath contains proportionately approximately 4 ounces of ammonium sulphate.

3. That improvement in the art of cadmium plating which involves the inclusion in 45 an appropriate bath containing cadmium oxide and sulphuric acid in the approximate proportions of 2½ ounces cadmium oxide

and 6 ounces sulphuric acid per gallon of water, of 1 to 10 grams of a disaccharide.

4. That improvement defined in claim 3 wherein the bath contains proportionately approximately 4 ounces of ammonium sulphate. 55

5. That improvement in the art of cadmium plating which involves the inclusion in an appropriate bath containing cadmium oxide and sulphuric acid in the approximate 60 proportions of 2½ ounces cadmium oxide and 6 ounces sulphuric acid per gallon of water, of 1 to 10 grams of commercial barley sugar.

6. That improvement defined in claim 5 wherein the bath contains proportionately 65 approximately 4 ounces of ammonium sulphate.

7. That improvement in the art of cadmium plating which involves the inclusion in an appropriate bath containing cadmium oxide and sulphuric acid in the approximate 70 proportions of 2½ ounces cadmium oxide and 6 ounces sulphuric acid per gallon of water, of 1 to 10 grams of commercial malt sugar. 75

8. That improvement defined in claim 7 wherein the bath contains proportionately approximately 4 ounces of ammonium sulphate.

In witness whereof, I, CHAD H. HUMPHRIES have hereunto set my hand at Indianapolis, Indiana, this 2nd day of April, A. D. one thousand nine hundred and twenty-eight. 80

CHAD H. HUMPHRIES.

85

90

95

100